

Sept. 27, 1938.

**G. A. BERRY**

2,131,702

## COAL PROCESSING

Filed Oct. 24, 1936

3 Sheets-Sheet 1

Fig. 1.



INVENTOR.

INVENTOR  
BY *George A. Berry,*  
*Robert James Morton*  
ATTORNEY.

Sept. 27, 1938.

G. A. BERRY

2,131,702

COAL PROCESSING

Filed Oct. 24, 1936

3 Sheets-Sheet 2



*Fig. 2.*

SOLID RATE = X  
GAS RATE = Y



SOLID RATE = X  
GAS RATE = Y- $\alpha$   
BUT TOTAL HEAT INPUT  
SAME AS IN (2)



SOLID RATE = X  
GAS RATE = Y+ $\beta$

INVENTOR.

GEORGE A. BERRY  
BY *Robert Anne Norton*  
ATTORNEY.

Sept. 27, 1938.

G. A. BERRY

2,131,702

COAL PROCESSING

Filed Oct. 24, 1936

3 Sheets-Sheet 3

*Fig. 4.*



$$\text{SOLIDS RATE} = \frac{X}{4} \quad \text{GAS RATE} = \frac{Y-a}{4}$$

BUT MAXIMUM RATE OF TEMPERATURE RISE IS SAME AS IN (2)

*Fig. 6.*



INVENTOR.  
BY *George A. Berry*,  
*Robert Lewis Morton*  
ATTORNEY.

## UNITED STATES PATENT OFFICE

2,131,702

## COAL PROCESSING

George A. Berry, Bound Brook, N. J., assignor to  
 National Fuels Corporation, Bound Brook,  
 N. J., a corporation of New Jersey

Application October 24, 1936, Serial No. 107,336

6 Claims. (Cl. 202—20)

The object of this invention is broadly to transform bituminous coal into a carbonizing fuel resembling anthracite and to recover other valuable products. More particularly, the invention is concerned with producing carbonized briquetted fuel of high density.

This invention is in part a continuation of my copending application Serial No. 680,026, filed July 12, 1933.

10 By this invention, very valuable commodities may be recovered from bituminous coal, and particularly from the so-called "slack" which is produced in large quantities in the mining and transportation of bituminous coal and which sells 15 for considerably less than the price of prepared sizes of bituminous coal. The invention is not limited to the treatment of coal in the form of slack, but is applicable to run of mine coal and prepared sizes.

20 The solid product of the present invention is characterized by the following properties:

1. It is hard or harder than anthracite and has such a high density that the specific gravity is 1.1 or higher so that adequate weight of fuel 25 can be put in a fire box of given volume.

2. The product ignites more readily than anthracite coal and burns at an even rate.

3. The product sustains combustion at temperatures lower than anthracite and is smokeless. It will burn uniformly throughout the fire 30 bed and does not tend to go out around cooled sides as is the case with anthracite.

4. The ash content is low and the calorific value per unit weight is high.

35 The process of this invention is further characterized by a high yield of organic vapors condensable at ordinary temperatures and in primary condition; that is to say, substantially of the same composition as they were when first 40 evolved from the coal, and hence substantially unchanged by cracking. Gases uncondensable at ordinary temperatures, and having high calorific value are also recovered, and when using one modification of the invention, a second gas of 45 lower calorific value can be separately removed from the process.

These products may be produced from a wide variety of grades or characters of bituminous coal, of which, for example, the coal fields of 50 eastern United States afford a practically unlimited supply.

The process is carried out continuously, preferably with a countercurrent flow of gases and solids. It is preferred to grind the coal and 55 form it into briquettes, although the invention is

not limited to the treatment of the material in briquette form. The degree of grinding which is necessary will vary with different coals, but should be sufficient to permit operation without swelling under the controlled heating conditions 5 which will be described below, so that the final product will have a high specific gravity.

The sizes of the coal particles used in forming the briquettes are also such as will, in the formation of the untreated briquette, permit the 10 attainment of a high initial density therein which favorably influences the ultimate density of the finished product and favors the production on the carbonized briquettes of a smooth, clean exterior free from loose particles that 15 might rub off.

Different sorts of binder may be used, but binder consisting principally of organic material is recommended. It has been found advantageous to use a binder such as waste liquid 20 from the sulfite pulp process of paper making, commonly known as "sulfite liquor"; although other binders, such as starch or other carbohydrate material may be used. With some coals, such as semianthracite, bituminous binders such 25 as coal tar, pitch, etc. may be used.

The coal briquettes are heated up to final carbonizing temperatures of 700 to 1000° C. and then cooled down or quenched so that they can be discharged into the atmosphere without ignition. This heating may be considered as divided into three stages or temperature ranges, although, of course, it is not necessary to physically separate the stages. Heating and cooling 30 take place in all stages by contact of the 35 material with a gaseous medium of suitable temperature. The gaseous medium is substantially nonreactive with the coal and with the products which it gives off. The stages are as follows:

1. The first stage involves heating the coal 40 or briquettes up to a temperature of about 300 to 350° C. at which temperature tar vapors and condensable hydrocarbons will appear. The upper limit of this first stage or temperature range is determined by the sort of coal treated.

2. The second stage is the low temperature distillation stage and extends from the 300 to 350° temperature at the end of the first stage up to 500 to 600° C. It is during this stage that most of the vapors, condensable at ordinary temperatures are likewise produced.

3. The third stage is the final carbonization and extends from the upper temperature limit of the second stage up to 700 to 1000° C. Further amounts of tar vapors are evolved during 55

this stage, together with a permanent gas of lower calorific value, and the briquette shrinks more and more and acquires increased density and hardness. The final temperature will depend on 5 the reactivity and density desired in the final product. A lower final temperature will give a more easily ignitable less hard and dense product which is suitable for fire place, brazier and similar methods of heating. On the other hand, 10 a higher final temperature will give a harder and denser product suitable for furnace firing.

4. The fully carbonized coal or briquettes are then cooled in a current of nonreactive gas down to a sufficiently low temperature so that they can 15 be discharged into the atmosphere without ignition and can be readily handled.

I have discovered that difficulties which have hitherto been encountered in coking bituminous coal and particularly briquettes made from such 20 coal, have been due to the fact that bituminous coal becomes plastic during the second stage referred to above, and that if the heating is too rapid, the vapors evolved in the interior of the lumps or briquettes cannot reach the exterior 25 readily and therefore tend to swell the briquette and produce a porous final product which does not have the requisite density for satisfactory fuel use. I have found that the critical points in carbonizing lie in the second stage. The most 30 critical points do not extend throughout the whole range of this second stage, but are located usually at certain temperatures which vary somewhat with different coals. Thus, in the first stage the heating may be very rapid, for example, 35 heating increments per minute of  $10^{\circ}$  C., or even higher, do no harm and the same is true in the third stage. It is only necessary to control the rate of heating accurately in the second stage and in this control it is not sufficient that the 40 average rate of heating during the second stage be below the critical point. The rate of heating will depend on the coal used and on the binder used, and to some extent on the fineness of grinding of the coal where briquettes are made. In 45 general, it will vary from about  $1\frac{1}{4}$  C. per minute for badly swelling or softening coal, up to nearly 10 C. per minute with certain coals such as Pocahontas and New River coal, which do not swell badly or soften unduly. The proper maximum 50 rate of heating will vary with the nature of the coal, and the average rate of heating throughout the stage will also vary with the amount of heating gas circulated per unit of weight and time which will be brought out in 55 greater detail below in connection with the description of Figs. 2 to 6 of the drawings.

In the process of the present invention, the coal or briquettes pass through the different temperature zones or regions, for example, by passing 60 downwardly through a retort countercurrent to the heating and cooling gas or gases for the various stages. Of course, any other means which will move the coal or briquettes countercurrent to the gas stream may be employed and 65 the present invention is not concerned with any particular structural details of retort design. In general, the average rate of heating through the critical zone will depend on the rate at which 70 the briquettes pass through the zone, provided the flow of heating gas and its heat content are such as to supply the heat required to raise the briquettes to the final temperature of the zone. The maximum rate of heating occurring at any 75 point in the zone will, however, also depend on

other factors, notably, ratio between the weight of heating gas and briquettes.

The invention will be described more particularly in conjunction with the drawings in which:

Fig. 1 is a diagrammatic illustration of a plant 5 for carrying out the present invention using a plurality of heating gas circuits; and

Fig. 2 to Fig. 6 are curves of gas and coal temperatures for various gas ratios and coal feeds.

In its broader aspects, the present invention 10 is not concerned with the particular nature of the heating and cooling gas used so long as it is substantially nonreactive with the coal or with its distillation products, although in the preferred embodiment which will be described below in 15 connection with Fig. 1 of the drawings, the evolved gases themselves are used as nonreactive gases and different gas circuits are used for the different stages in order to recover the high calorific, permanent gas separate from the lower calorific 20 gas produced in the final carbonizing zone or stage. While this preferred embodiment represents important practical advantages because of the higher price which can be obtained for undiluted, high calorific, permanent gases, the invention 25 is broadly not limited to this procedure. If desired, a nonreactive gas stream may flow countercurrent to the coal throughout the whole length of the retort. In more specific aspects, 30 of course, the preferred embodiment constitutes a part of the present invention.

The heating gas performs two functions: First, it is a very uniform heating medium, contacting the surfaces of all of the lumps or briquettes, and secondly, the large volume of gas which is, 35 of course, necessary because of the low specific heat per unit volume, sweeps or scrubs off the vapors reaching the surface of the coal. The partial pressure of the evolved vapors is therefore very low and they remain volatile at temperatures far below their boiling point at atmospheric pressure, and hence do not show any tendency to condense or precipitate on cooler coal which they encounter in passing countercurrent through the stage.

Since the vapors do not encounter solids at higher temperature, there is practically no tendency for the vapors to crack after evolution. This is a very important feature of the present invention and one which can not be achieved by other means of heating such as external heat, radiant heat, and the like, because there the vapors distilling out from the coal or briquettes distill at atmospheric pressure or a little below and, therefore, when they encounter cooler coal they tend to condense on the surface, which leads to serious difficulties, or the vapors encounter the hot source by heat and crack. The partial pressure of the evolved vapors will, of course, vary with the nature of the coal. Usually very high volatile coal will evolve more vapors for a given amount of heating gas and therefore will exhibit a slightly higher partial pressure than a lower volatile coal. The pressures are, however, very low, even for high volatile material, and are of the order of 55 magnitude of 20 mm. of mercury or less.

This second function of the gas, namely, the rapid sweeping away of vapors evolved by the coal and under partial pressures much lower than the atmosphere, is one of the most important factors in the present process. Internal gas heating is therefore in no sense the equivalent of other forms of heating. It is thus possible to avoid swelling of briquettes when heating is by means of a gas stream, even though this rate is suffi- 75

ciently high so that the briquettes would swell if the heating took place by other means which would not permit removal of the evolved vapors at a lower partial pressure.

- 5 From an economic and practical standpoint, the relative amount of gas used in heating is vital. This is clearly shown in Figs. 2 to 6 of the drawings which represent curves, the abscissae being temperatures and ordinates time.
- 10 Fig. 2 shows the ideal and preferred operating conditions of the present invention. In this figure the weight of heating gas circulated per unit of time multiplied by its specific heat is exactly equal to the weight of coal or briquettes multiplied 15 by their apparent specific heat. The expression "apparent specific heat" is used because the amount of heat absorbed by a unit weight of coal or briquettes in passing through the second stage does not necessarily correspond exactly to the 20 actual specific heat of the material multiplied by the temperature rise. The reason for this is that there are other phenomena taking place, such as cracking, distilling of vapors and the like, which reactions may be either endothermic or 25 exothermic and which will vary in amount and to some extent in nature with different coals. Thus, the amount of heat required to bring a given initially-introduced weight of briquettes from the entering temperature up to the exit 30 temperature divided by the temperature rise and the weight of the material will give a figure of apparent specific heat which takes in account all of the thermodynamic factors involved.

As an example, a given coal may show an apparent specific heat of about .3 and a given heating gas may have a specific heat of about .4. In such a case, in order to have the same heat capacity, the weight of gas circulated per hour must be  $\frac{3}{4}$ ths the weight of the briquettes passing 40 through the zone. In such a case, when the entering gas is approximately at the exit temperature for the zone, the curves for gas temperature and coal temperature will be two parallel straight lines displaced by the small difference 45 required for the heat head to transfer heat from the gas to the solid. It will be apparent that the rate of heating at all points is the same and is defined by the slope of the curve with respect to the abscissa or mathematically expressed, is equal 50 to the first derivative of the curve.

Fig. 3 shows the conditions which obtain when the ratio of gas to solids is decreased. In order to introduce the same total quantity of heat to bring up all of the briquettes to the exit temperature of the zone, it is, of course, necessary to introduce the gas at a higher temperature. It will be apparent from a consideration of the curves which are no longer straight lines that the rate of heating in the upper part of the zone is 55 less than the average and the rate of heating in the lower part of the zone is greater than the average; and that as compared to Fig. 2 a given temperature is reached at a later time, which means in the case of a vertical retort at a lower 60 point. Assuming that for a given coal the rate of heating shown in Fig. 2 is the maximum permissible, it will be obvious that if conditions are changed as shown in Fig. 3 the rate of heating in a portion of the stage will exceed the permissible maximum. In other words, the process will 65 not work and the coal will swell.

Fig. 4 shows how this condition can be compensated for. In Fig. 4, the ratio between gas and solids is kept constant at the same ratio as 70 Fig. 3, but the rate of flow of the solids and con-

sequently, of course, the total rate of flow of the gas, is greatly decreased which is shown by a longer time for the cycle appearing as a higher ordinate on the curve and correspondingly a lower average heating rate. If the unbalance between gas and solids is not too great, it is possible, as is shown in Fig. 4, to so reduce the average rate of heating that the maximum anywhere along the curve does not exceed the permissible rate set by the conditions in Fig. 2. Thus, as 10 far as rate of heating is concerned, Fig. 3 shows that it is possible to obtain the required rate of heating without balancing the heat capacity of the gas and solids accurately but this is obtained only at the sacrifice of output because in order 15 to keep the maximum heating rate within the permissible limitation, the average heating rate, which determines the output of the equipment, must be greatly reduced.

If the relative amounts of gas and solids are 20 unbalanced in the opposite direction, that is to say, if the amount of gas is greater than that corresponding to the heat capacity of the briquettes, a condition obtained as shown in Fig. 5. Here, again, the gas and solids temperature 25 curves are no longer straight lines but instead of the rate of heating being lower than the average in the upper portion of the zone, and higher than the average in the lower portion of the zone, it is higher in the upper portion of the 30 zone and lower in the lower portion. In this case, again, if the conditions of Fig. 2 represent the maximum permissible heating rate, the maximum rate in the upper part of the zone as shown in Fig. 5 will exceed this figure and therefore 35 again the process will not work and the coal will swell.

Fig. 6 shows how it is possible to compensate for the unbalance in Fig. 5 and again the unbalance is compensated for by decreasing the 40 rate of flow of briquettes and gas in the same proportion and therefore decreasing the average rate of heating to a point sufficiently low so that the maximum rate does not exceed the permissible figure. Again, as in Fig. 3, the compensation 45 is obtained at the expense of a longer time cycle and greatly decreased output for a given piece of equipment.

The compensation shown in Fig. 3 is further complicated by the fact that there is another 50 factor involved in the practical carbonization of briquettes by the present process, and this is the factor of head load which the briquettes can sustain. As the coal reaches its point of maximum plasticity or fluidity, there is a tendency 55 for the briquettes to become deformed or stick together and for any given coal and any given binder briquettes will stand a certain maximum head load at the point of greatest plasticity. The reason for avoiding any considerable deformation of any sticking together of the briquettes lies in the necessity for subjecting the surface of the briquettes during the carbonization cycle to free and uniform contact with the heating gases. If briquettes are not deformed 60 excessively and do not stick together, they roll sufficiently in passing through the retort so that the points of contact between the briquettes are constantly shifted.

In general, the plasticity increases as the briquette passes through the critical zone reaching a point of maximum and then again decreases. If we assume a point of maximum plasticity occurring at a certain temperature on the curve in Fig. 2, and where the preferred practical de- 75

sign of vertical retort is used this represents a certain depth, there will be a corresponding head load at this point. If Fig. 2 is compared with Fig. 3, it will be apparent that the same temperature is reached at a lower point because the rate of heating is slower in the upper portion and faster in the lower portion, and all temperatures are therefore displaced downwardly in the column of coal or briquettes. If Fig. 2 represents 10 the maximum permissible head load at the point of greatest plasticity, it will be obvious that Fig. 3 will cause failure because the head load will be increased and reduction in the rate of flow which is used to compensate in Fig. 4 will not help 15 because the briquettes will merely flow more slowly but still the same temperature will be reached at the same height in the column. It becomes necessary, therefore, where the gas-briquette ratio is unbalanced by having too little 20 gas, to modify the design of retort by increasing its horizontal dimensions in order to permit compensation for gas-solids unbalance. Other means for decreasing head load may also be used.

25 From the above, it will be apparent that the balancing of gas to solids in the critical zone is of the greatest practical importance and that where the balance is perfect, operation can take place at maximum output. The control is best at 30 perfect balance because slight variations will have less effect than under conditions shown in Fig. 3 for the reason that there gas temperature and solids temperature do not run along parallel lines and there is greater heat head which permits considerable fluctuations in the rate of 35 heating. This substantially accurate balancing of gas and solids heat capacity is the preferred embodiment of the present invention. Small deviations from the optimum can be compensated 40 for and in its broader aspects, the invention is therefore not limited to obtaining perfect gas-solids balance, and a certain amount of unbalance can be tolerated if the output is kept sufficiently low.

45 Another advantage of the preferred specific embodiment of the present invention represented by Fig. 2 is that the heat head between gas and solids is kept at a minimum. Both Figs 3 and 5 show at one or other ends of the curves a much larger heat head or heat difference between gas and solids. There is thus greater danger of cracking or carbonization of vapor evolved at the surface of the coal when encountering the much hotter gas at levels of the zone 50 where the gas temperature and solids temperature curves diverge widely.

Heating by means of a gas stream also results in great uniformity and since the critical factor of rate of heating applies to each individual coal 55 lump or briquette it is not sufficient that the rate of heating in the critical stage be low merely for the charge as a whole because it is not the average condition throughout the charge which counts but the condition at the surface of each lump. Gas heating, therefore, gives a uniformity throughout the whole charge which is impossible with external heating.

While the present invention usually finds its 60 most attractive economic field in the carbonizing of relatively cheap bituminous coals, particularly in the form of briquettes, it should be understood that the invention is not limited to treating a uniform material. On the contrary, blends or 65 mixtures of different kinds of bituminous coal or 70 bituminous coal with anthracite, semianthracite,

semibituminous, lignite, semicoke and coke may be used. This is particularly important where fine noncooking refuse is available such as, for example, coke breeze, anthracite fines, for example anthracite fines obtained as the flotation concentrate from the flotation cleaning of anthracite slush culm. These fine materials command a very low price and can be effectively blended with bituminous coal by means of the present invention to produce high grade briquettes having superior burning characteristics. 10

The operation of the invention will be described in detail in connection with a typical example using Pocahontas or New River coals and using the referred dual circuit heating system of 15 Fig. 1. It will be understood, of course, that the rates of heating apply only to these coals and will vary with other coals and for each coal the optimum rates must be determined by experiment.

In Fig. 1 of the drawings the reference character 1 indicates a vertically disposed, elongated, heat insulated retort with a chamber 2 at its upper portion to admit briquettes or lumps of coal without permitting escape of gases, and with a valve 3 at its lower end to permit discharge of the 20 final solid or carbonized product without permitting escape of gases.

The retort 1 may be regarded as divided into four sections 4, 5, 6 and 7, acting as preheating, distilling, high temperature, and cooling or 30 quenching sections, respectively.

The high temperature section 6 may be a retort of refractory material or metal and may be surrounded by a heating device 8. A burner or burners 9 are provided for the heating device 8. 35 An air inlet for the burner is shown at 10 and a lean gas inlet pipe 11 is provided with a valve 11' leading to this burner. The products of combustion from the burner or burners pass into an annular combustion space or flue 12 in the heating device 8. Ports 13 lead from the combustion space 12 to the annular space 14 from which a series of exits or outlets 15 for hot products of combustion lead into the lower portion of the high temperature section 8. 45

A pipe 16 provided with a valve 16' leads to a manifold 17 at the lower portion of the cooling section 7. A series of openings 17' lead from the manifold 17 into the section 7.

An outlet 18 from the space 19 at the upper end 50 of the high temperature section 6 leads to the heating side of the heat exchanger 20. A pipe 21 leads from the heat exchanger 20 to the condenser 22 that may be of any suitable type to remove easily condensable products from the gases. A pipe 23 leads uncondensed gases from the condenser 22 to the suction pump or blower 24 from which a pipe leads to the tar extractor 25 which may be any of the well known suitable types. A pipe 25' for gases from which tar has been removed leads from the extractor 25 to the lean gas receiver 26. A valved outlet or vent pipe 27 is provided on the receiver 26. The valved pipes 11 and 16 also are connected to the lean gas receiver 26. 60

A pipe 30 leads from the heated side of the heat 65 exchanger 20 to a manifold 31 at the lower portion of the distilling section 5 of the retort 1, from which manifold 31 hot gases pass through the openings 32 into the lower portion of the distilling section 5. An outlet pipe 33 leads from the upper portion of the distilling section 5 to the condenser 34 which removes organic liquids that are condensable at ordinary temperatures. A pipe 35 leads uncondensed gases of high calorific 70 power from the condenser 34 to the suction pump 75

or blower 36 from the outlet of which pipe leads to the tar extractor 37 of any of the well known types suitable for removing tar. A pipe 37' for rich gases from which tar has been removed leads from the extractor 37 to the receiver 38 which is provided with a valved outlet 39 for surplus rich gas. A valved pipe 40 leads rich gases from the receiver 38 to the heat exchanger 20 where these gases are heated and pass into the distilling section 5 through the pipe 30. A valved by-pass 41 around the heat exchanger 20 leads from the pipe 40 to the pipe 50 to provide convenient regulation of the temperature of the rich gases that enter the distilling section 5 through the pipe 30.

15 An outlet pipe 44 leads from the upper portion of the preheating section 4 to the suction pump or blower 45, from the outlet of which a valved pipe 46 leads to a condenser 47 from which a pipe 47' leads uncondensed gases to the heater 48. The 20 gas heater may be heated by combustion of lean gases taken from the receiver 26 through the valved pipe 49 to a burner 50, air for combustion purposes being admitted through the inlet 51. The hot products of combustion from the burner 25 50 after heating the gas heater 48 are lead by the pipe 53 into the lower portion of the preheating section 4. A valved pipe 54 leads from the lean gas receiver 26 to the pipe 44 to supply any needed make up gases for the preheating section.

30 The volumes of the gases and the amount of the gas made in the several sections of the retort depend upon the type of coal being treated, although the difference between coals from the standpoint of gas volumes required for heat 35 transfer purposes from the gas to the coal is small. However, differences in coals will affect to a considerable extent the amount of gas produced in the several sections of the retort and the weight of the finished product for a given 40 weight of raw coal treated.

For example, coal containing approximately 20% of volatile matter will produce amounts of gas and will require rates of gas circulation and temperatures as follows:

45 When 2000 lbs. of such coal is treated by this invention approximately 26,000 cubic feet of lean gas from the receiver 26 will be required in the quenching or cooling section 7. This lean gas will have a temperature of approximately 900° C. when it reaches the lower portion of the high 50 temperature section 6, which is approximately the temperature of the carbonized product at this point. Approximately 43,000 cubic feet of gas is required in the high temperature section 6. This 55 is made up of the 26,000 cubic feet from the section 7 plus 17,000 cubic feet of gaseous products of combustion from the combustion flue 12. The lean gas entering through the pipe 15, and the products of combustion from the combustion flue 12 passing through the high temperature 60 section 6 is augmented by approximately 6,000 cubic feet of gas evolved from the material being treated in this section, thus making approximately 49,000 cubic feet of gas leaving the high temperature section 6. The gas entering the high temperature section 6 from the combustion flue 12 is taken from the lean 65 gas receiver 26, and is caused to undergo a sufficient amount of combustion to bring the temperature of the mixture to slightly above 900° C., the volume being about 13,300 cubic feet. The 70 temperature of the gas leaving the upper portion 75

of the high temperature section 6 through the pipe 16 is about 100° higher than the solid products at this point in the retort 1.

About four-fifths of the gas passing through the high temperature section 6 may pass out through the pipe 18 to the heat exchanger 20, condenser 22, tar extractor 25 and into the receiver 26. About one-fifth or 9,700 cubic feet of the gases passing through the high temperature section 6 may pass into the lower portion of the distilling section 5 at a temperature of about 600° C. and be joined by heated rich gas entering this section through the pipe 30. By means of the vent 27 on the lean gas receiver 26 the amount of gas that passes from the high temperature section 6 to the distilling section 5 can be regulated, thus varying the amount of lean gas that is blended with the distilling zone gas so that the heating value of the surplus rich gas that is produced in the distilling zone can be controlled to suit the use to which this rich surplus gas is to be put.

When it is desired that the gases evolved in the distilling section 5 be not contaminated with gases from the sections 6 and 4, the process can be readily operated to prevent this. Gas tight gates to permit passage of the coal may be located at the ends of the section 5 for this purpose. As already explained, a portion of the lean gas from the receiver 26 may be used for combustion purposes in the gas heater furnace 50 and some of it may be passed through the pipe 54 and used to augment the gas circulated through the preheating section 4.

When treating a ton per hour of the coal mentioned above containing about 20% of volatile matter, approximately 34,000 cubic feet of gas is introduced into the lower portion of the distilling section 5 and is augmented by approximately 4,000 cubic feet evolved from the material being treated so that approximately 38,000 cubic feet of gas leaves the upper portion of the distilling section 5. The rich gas which is made in the distilling section 5 and recirculated by being caused to enter through the pipe 30 is heated to 45 a predetermined temperature which depends upon the upper limit of temperature at which the coal being treated is no longer in a plastic condition and has lost its tendency to swell if heated at a rapid rate. The gas entering through 50 the pipe 30 augmented by the lean gas from the high temperature section 6 and also by the gas evolved from the material in this section should be just sufficient in quantity to transfer its heat to the material being treated in this section and 55 raise its temperature to within a few degrees of the temperature of the gas entering through the pipe 30, which is approximately 500° C. The amount of gas passing through the distilling section and the material being treated passes 60 through at such a rate that a temperature gradient of a straight line order is produced so that there is a practically constant increase in temperature per unit of vertical length so that the temperature rise per unit of time is not so great 65 in this section as to produce swelling of the material, or deformation and sticking.

The rich gas of high B. t. u. value is drawn off through the pipe 33 and is passed through the condenser 34 and tar extractor 37 to the gas receiver 38. The surplus is withdrawn through the valved pipe 39 and the portion that is recirculated passes through the pipe 40 and heat exchanger 20 (or part of it through the by-pass 41) back to the lower portion of the distilling section 5. The 75

temperature may be regulated by by-passing the desired amount through the pipe 41.

With the coal under consideration approximately 33,000 cubic feet of gas is passed through the preheating section 4, the gas entering the lower portion of this section through the pipe 53 having a temperature of about 300° C. This gas consists of gas given off by the coal while it is being preheated in the preheating section 4 plus some lean gas from the receiver 26, when necessary. Approximately 5% of the total amount of gas in this circuit is caused to pass downwardly into the upper portion of the distilling section 5 to prevent tar-laden gases from this section from entering the preheating section 4 and causing condensing and precipitating tars on the briquettes in this section. The remaining portion of the gas from the gas heater 48 raises the temperature of the raw material to about 300° C. as it leaves the lower portion of the preheating section 4 and removes from this raw material any moisture or other material that would be volatilized at the temperature to which the material is subjected in this preheating section. The moisture and other condensable products are condensed out of the gas leaving through the pipe 44 before it enters the heater 48.

The rich gas that is produced by the coal in the distilling section 5 is of very high calorific value. It has been found to be from 800 to 1000 or more B. t. u. per cubic foot, depending upon the sort of coal that is treated. This gas is largely methane and higher hydrocarbons, usually called illuminants and a relatively small amount of hydrogen.

In the above example the rate of heating in the distilling section is 2 to 4° C. per minute for the coals specified.

The invention has been described specifically in conjunction with a plurality of gas circuits which permit the separate removal of high calorific gas. It will be apparent that the carbonization, that is to say, the production of the solid product of the invention is not concerned with the characteristics of heating gas so long as the heating gas is nonreactive with the material. Where it is not desired to obtain high calorific permanent gas separately, a cheaper operation from the standpoint of equipment and operating costs can be effected by permitting the gas stream to flow through the whole length of the retort. This will result in mixing the lean gas present in section 6 with the rich gas evolved in section 5 and the whole will be diluted with the amount of nitrogen introduced by the combustion of a portion of the gas in the combustion flue 14. Where the gas from section 6 is used as the heating gas for section 5, it is unnecessary and, in fact, undesirable for the gas to leave section 6 at a temperature of 100° above that of the solids. On the contrary, it should leave at approximately the temperature of the solids as they emerge from section 5. This is effected by reducing the volume of gas circulated through section 6 to that which circulates through section 5 when a dual system is employed, and also by reducing the proportion of gas burned in the burners 9 because there is no longer any need to compensate for the radiation and other losses involved in the heat exchanger 20 and the whole heating gas circulating circuit of section 5 which is external to the retort.

Both of these factors reduce dilution because not only is the volume of lean gas entering section 5 lower, but the gas is not as lean, that is to say,

it is not diluted with as much nitrogen and other inert.

Compromises may also be effected, that is to say, distilling section 5 may be partly heated by gases flowing up from the section 6 and partly by gases coming from the heat exchanger 20. When such a compromise is employed the condenser 22, tar extractor 25, and receiver 26 is reduced in size by corresponding reduction in the heat losses and in the power and other operating expenses. The gas taken off through the pipe 39 will, of course, be of a calorific value intermediate between that obtainable with a full dual circuit operation and that corresponding to a complete single circuit. In every such case, the skilled engineer will choose a compromise which represents the best economic value for a particular plant using a particular raw material in a given location. It is an advantage of the present invention that gases of different calorific power can be produced so as to adapt the process for the different conditions obtaining in different geographic locations.

In the specific description of the invention in connection with Fig. 1 of the drawings, reference has been made to zones which in the retort shown in the drawings are equally physically distinct compartments. It should be understood however that this particular apparatus structure forms no part of the invention and the zones as referred to in the claims are directed entirely to the temperature ranges through which the coal passes, regardless of whether the zones are physically separated or simply temperature ranges in a single moving column. It is, of course, possible to break up the zones into physically separate retorts where the structural design and space requirements make such a construction desirable. The invention, of course, covers the process of heating the coal at the rates and with the gas volume specified, regardless of the physical location of the various heating zones.

The invention has been described in conjunction with the use of gas heating for all stages or zones. This is, of course, the preferred and ideal method, but it should be understood that gas heating is essential only in the second stage or zone where the controlled heating and rapid removal of evolved vapors are required. It is therefore possible, although less desirable, to heat in the first or third zones by other means than a gas stream and such modifications are included in the broader aspects of the invention. Such modifications are, however, normally less desirable and accordingly, the preferred embodiment of the invention which represents the most efficient practical method of carrying out the principles of the invention, utilizes gas heating for all three zones.

In the claims the term "capable of coking" is used to define coals which pass through a plastic state on heating and are therefore capable of forming an autogenous binder during carbonization. It should be understood that this term is not used in a narrow sense in which the term is sometimes used in the art to designate a type of coal which is capable of practical economical coking in the ordinary type of externally-heated by-product coke oven. Wherever the term is used in the claims, it is used in the broader sense defined above and in no other sense.

I claim:

1. A continuous process of destructively distilling coal which comprises passing the coal capable of coking in succession through a series of

zones, the first being a preheating zone to a temperature at which evolution of volatile material begins, the second zone being the first distilling zone and extending from the softening point of the coal up to a temperature of about 500 to 600° C. in which zone the major portion of the condensable hydrocarbon volatiles are evolved and a third zone extending up to about 700 to 1000° C. in which zone the desired degree of distillation and carbonization is reached, the heating for at least the second zone being by contact with hot gases which are substantially nonreactive with the coal at the existing temperatures in the zones, the volume of heating gas and its specific heat in the second zone being sufficient so that when introduced at substantially the exit temperature of the coal leaving the zone it contains sufficient heat to bring the coal passing through the zone up to exit temperature while being itself cooled down to substantially the temperature of the coal at the inlet of the second zone, the rate of heating in the second zone being sufficiently low so that the particular coal will not swell sufficiently to produce a product having a density as light as high-temperature coke produced from the same coal in a standard by-product coke oven.

2. A continuous process of destructively distilling coal capable of coking which comprises grinding the coal, incorporating a binder with the ground coal forming it into briquettes having sufficient strength to permit handling and passing the coal in succession through a series of zones, the first being a preheating zone to a temperature at which evolution of volatile material begins, the second zone being the first distilling zone and extending from the softening point of the coal up to a temperature of about 500 to 600° C. in which zone the major portion of the condensable hydrocarbon volatiles are evolved and a third zone extending up to about 700 to 1000° C. in which zone the desired degree of distillation and carbonization is reached, the heating for at least the second zone being by contact with hot gases which are substantially nonreactive with the coal at the existing temperatures in the zones, the volume of heating gas and its specific heat in the second zone being sufficient so that when introduced at substantially the exit temperature of the coal leaving the zone it contains sufficient heat to bring the coal and binder passing through the zone up to exit temperature while being itself cooled down to substantially the temperature of the coal at the inlet to the zone, the rate of heating in the second zone being sufficiently low so that the particular coal will not swell sufficiently to produce a product having a density as light as high-temperature coke produced from the same coal in a standard by-product coke oven.

3. A continuous process for destructively distilling coal capable of coking which comprises passing the coal in succession through a series of zones, the first being a preheating zone to a temperature at which evolution of volatile material begins, the second zone being the first distilling zone and extending from the softening point of the coal up to a temperature of about 500 to 600° C. in which zone the major portion of the condensable hydrocarbon volatiles are evolved and a third zone extending up to about 700 to 1000° C. in which zone the desired degree of distillation and carbonization is reached, the heating for all zones being by contact with hot gases which are substantially nonreactive with the coal at the existing temperatures in the zones, the volume of heating gas and its specific heat in the second zone being sufficient so that when introduced at substantially the exit temperature of the coal leaving the zone it contains sufficient heat to bring the coal and binder passing through the zone up to exit temperature while being itself cooled down to substantially the temperature of the coal at the inlet to the zone, the rate of heating in the second zone being sufficiently low so that the particular coal will not swell sufficiently to produce a product having a density as light as high-temperature coke produced from the same coal in a standard by-product coke oven.

4. A process according to claim 1 in which the heating in the third zone is effected by a gas stream of relatively low calorific value which has been partially burned and the heating in the second zone is effected by the circulation of a gas stream of high calorific value whereby dilution of the volatile material evolved in the second zone with gases of low calorific value is avoided.

5. A method according to claim 1 in which the heating in the preheating zone and in the third zone is at a sufficiently high rate so that the total time cycle for carbonizing through the three zones is less than the normal cycle of standard modern by-product coke ovens of the externally heated type.

6. A method according to claim 2 in which the heating in the preheating zone and in the third zone is at a sufficiently high rate so that the total time cycle for carbonizing through the three zones is less than the normal cycle of standard modern by-product coke ovens of the externally heated type.

GEORGE A. BERRY. 55